# EUROPEAN PATENT APPLICATION

(11) **EP 2 154 467 A1**
(43) Date of publication of application: **17.02.2010**
(21) Application number: 08105040.3
(22) Date of filing: 14.08.2008
(51) Int. Cl.: F28F 19/02, B05D 7/14, B05D 7/00

(54) **Heat exchanger with coating, and process for its manufacture**

(71) Applicant: BSH Bosch und Siemens Hausgeräte GmbH, 81739 München (DE)
(72) Inventor: Grunert, Klaus, 13465, Berlin (DE); Pietsch, Harald, 12683, Berlin (DE); Castillo Fernandez, Jose Luis, 31.300, Tafalla (Navarra) (ES); San Martin Sancho, Roberto, 31200, Estella (ES)

(57) **Abstract**

The invention relates to a heat exchanger being coated at least partially with a polymer coating on a part of a surface of the heat exchanger. The part of the surface has a passivating layer interposed between said coating and said surface. The heat exchanger may be combined with a household appliance, particularly a dryer, to form a functional component, particularly a heat sink, of said household appliance. The invention relates moreover to a process for the manufacture of this heat exchanger.

## Description

The invention relates to a heat exchanger being coated at least partially with a polymer coating on a part of a surface of the heat exchanger and a preferred process for its manufacture.

A heat exchanger has to fulfill several requirements in order to effectively exchange heat. First of all, the heat conductivity of its body should be good. Moreover, a surface of a heat exchanger exposed to any kind of dirt or dust should be easy to clean since any dirt or dust adhering to the surface would tend to reduce the efficiency of a heat exchanger. This is especially true for a heat exchanger in a dryer that is commonly used for drying wet clothes.

German Patent Application 10 2008 010 517.1 filed February 22, 2008 and fully incorporated herein by reference discloses a dryer comprising a heat exchanger which has a polymer coating on a surface exposed to process air carrying small particulate matter, namely lint. Every heat exchanger operable as a heat sink in a dryer that recirculates process air to dry laundry is apt to be covered with lint, detergents and other particles that have passed a lint screen that is generally disposed upstream of the heat sink and thus stick to the exposed surface of the heat exchanger. Moreover, a heat exchanger in a dryer may come into contact with humidity at elevated temperatures. Under these conditions, lint, detergents and other particles tend to stick even better to the wet surface of the heat exchanger. These particles can be removed in principle by flushing with water. It is however useful if these particles do not stick too strongly to the surface.

The cleaning of a heat exchanger in a dryer generally depends on the type of the heat exchanger.

In general, a dryer for drying humid laundry contains as drying chamber a rotatable drum to contain the wet laundry, and additional air passages, in which process air may be circulated. Prior to entry into the drying chamber, the process air is heated by a heat source, so that it can absorb humidity from the laundry which may be tumbled in the drying chamber. After passing through the drying chamber, the process air is loaded with humidity, but also contains fine particles released from the laundry and specified as lint or fluff in general. It first reaches a lint filter or fluff filter, whereon these fine particles are predominantly collected, and then a heat sink where the process air is cooled. During this cooling process, the humidity condenses and is separated from the process air. From the heat sink, the process air flows back to the heat source where it is reheated and led back into the drying chamber. Although the fluff filter catches and retains a significant proportion of the fluff, the heat sink is nevertheless also noticeably loaded with the finest particles which the fluff filter cannot collect. That load may become relatively high because the fluff is deposited on and more or less sticks to the surface of the heat sink facing the process air, a process to which the condensed water in the heat sink contributes significantly.

An air-to-air heat exchanger for use as a heat sink is generally designed that it may be easily detached from the remainder of the dryer once one or more drying processes are completed. Cleaning can then be easily effected by rinsing with water. The situation is different if the heat sink is part of a heat pump. Dryers for drying laundry using a heat pump are disclosed in the documents WO 2007/093461 A1, WO 2007/093467 A1, and WO 2007/093468 A1, according to which the cleaning of the heat exchanger involves the use of brushes and additional liquid.

If the heat sink is part of a heat pump wherein the heat removed from the process air in the heat sink is pumped to the heat source to be used to heat the process air once again, it is in general not possible to have an easily detachable heat sink. For example, the compressor-type heat pump specified below connects the heat sink and the heat source in a heat transport circuit wherein a working medium or refrigerant circulates, for example a fluorinated hydrocarbon compound. The working medium flows in liquid form to the heat sink where it evaporates by means of heat from the process air. The evaporated working medium is led to a compressor. There it is compressed and conveyed to the heat source where it becomes liquid by transferring heat to the process air. The liquid working medium reaches a throttle behind the heat source, for example a valve, a diaphragm or a capillary, where its internal pressure and temperature decreases, and moves back to the heat sink, thus completing the circuit. The working medium circuit should be completely sealed to its ambient in order to ensure a long lifetime. This is normally achieved by sealing all components and joints between them tightly by soldering or brazing. Removal of the heat sink from the dryer is thus in general not possible without damaging the heat pump. The same applies if the heat pump is a thermoelectric heat pump based upon the utilization of the Peltier effect.

The coating of a heat exchanger operable as a heat sink, in particular its fins (if present), should contribute to an easy cleaning of the heat exchanger. However, during the drying process the wet and hot process air stresses the coating (in general a polymer coating) such that unwanted effects as increasing the surface energy and delaminating the coating from the surface may occur. Particles can then stick much easier to the non-protected surface and might be more difficult to remove. In the case where the heat exchanger is made of aluminum, aluminum oxide may form which could contribute to the delaminating of the coating and an overall worsening of the surface characteristics. In the latter case, aluminum oxide could stem also from the transport of a heat exchanger under a salty atmosphere as may occur during a sea transport of a household appliance comprising the heat exchanger.

DE 103 30 744 A1 discloses a coating system based on a polysiloxane resin formed from hydrolysable silane with a high hydrolysis speed. This coating system provides functional coatings with different properties; it is in particular easily cleanable and highly scratch resistant and also suitable for substrates made of glass, ceramic, metal, stone and plastic. The coating system of "example 2" is described to provide a hydrophobic easy-to-clean coating using very little surface energy, on the basis of which dirt and liquids can only weakly adhere to the coating. Thus the coated surface does not become heavily soiled and is easy to clean.

Further examples for easy-to-clean coatings based on polysiloxane resins are disclosed in WO 2001/064 801 A1, in particular its Examples 2B, 9, 34, 39 and 40. The coating renders the surface dirt-repellent, scratch-resistant and in some cases resistant towards high temperatures. The use of the coating for the protection of masonry from unwanted graffiti and for corrosion-resistant and non-sticky cookware, ovens and other equipment is disclosed.

An object of the present invention is thus the provision of a heat exchanger with an improved coating which is particularly useful under the conditions which are encountered by a heat sink in a dryer, in particular a clothes dryer. Another object is the provision of a process to manufacture such heat exchanger.

This object is achieved by the heat exchanger and the process, respectively, of the respective independent patent claim. Preferred embodiments of the heat exchanger and the process are specified in dependent patent claims. It is noted that preferred embodiments of the heat exchanger correspond to preferred embodiments of the process, and vice versa, even if not explicitly mentioned herein.

The invention thus provides a heat exchanger being coated at least partially with a polymer coating on a part of a surface of the heat exchanger, wherein the part of the surface has a passivating layer interposed between said coating and said surface.

By providing the passivating layer, a well-defined and stable interface is provided for bonding the polymer coating to the surface. The passivating layer provides the surface with a chemical stability that surpasses the stability of the surface without any passivation, and will prevent oxidation or any other degradation. To make the passivating layer, a variety of compounds and formulations including phosphate and chromate compounds dissolved in appropriately composed liquid formulations is commercially available for this purpose.

In accordance with a preferred embodiment of the invention, the passivating layer comprises a chromium compound. Even more preferred, that chromium compound comprises Cr(lll) ions.

In accordance with another preferred embodiment of the invention, the coating has a surface energy not exceeding 40 mN/m, in particular not exceeding 30 mN/m.

The surface energy can be measured by dropping special inks that are pigmented liquids having special properties. The behavior of these inks on the surface to be examined can be used to determine the surface energy. The surface energy can be determined based on the extent to which a drop of such an ink runs on the surface or whether it remains as more or less ball-shaped drop on the surface.

The heat exchanger according to the invention can be made of a variety of materials, in particular of plastic or metal. Preferably the heat exchanger comprises a metal such as aluminum, magnesium or copper. More preferably, the heat exchanger comprises more than 90 % aluminum. In particular, the heat exchanger consists of aluminum.

The heat exchanger of the present invention is preferably obtainable by a process comprising the steps:
(a) pretreating at least the part of the surface to be coated with a detergent, phosphate and/or borate containing solution,
(b) rinsing the surface with water,
(c) treating the surface with a passivating agent to yield a passivating layer
(d) rinsing the passivated layer with water, and
(e) coating the passivating layer with a polymer.

For the coating, numerous polymers can be used as long as they allow the provision of a coating with a surface energy not exceeding 40 mN/m. For the present invention, however, a polymer coating was found to be particularly suitable that comprises a polysiloxane resin. Preferably, the polysiloxane resin is a polyester-modified methyl phenyl polysiloxane resin. Such coatings are of particular advantage in that they can be very thin and are at the same time scratch-resistant, in particular when they are applied on a pretreated heat exchanger surface. A correspondingly coated heat exchanger can be cleaned with ease, in general by rinsing with water.

In a preferred embodiment of the present invention, ceramic particles, more preferred ceramic particles with a size of approximately 50 nm, are suspended in the polymer coating. The term "ceramic particles" as used herein means particles from essentially inert oxides, hydroxides and the like. Such ceramic particles comprise or consist of in particular silicon dioxide, calcium hydroxide and/or aluminum oxide together with derivatives such as boehmite.

The polymer coating has preferably a thickness of from 1 µm to 50 µm, more preferably of from 1 µm to 10 µm and most preferably of from 1 µm to 5 µm. The thickness of this coating can be measured in particular by means of scanning electron microscopy.

In a particular embodiment of the heat exchanger and the dryer of the present invention, the polymer coating comprises a pigment, in particular a dye. The pigment is preferably selected such that it fluoresces in visible light when irradiated with ultraviolet light. This embodiment allows to easily control whether the polymer coating has been accomplished as desired.

Advantageously, the heat exchanger of the present invention thus contains suspended in the polymer coating a pigment that fluoresces in visible light when it is irradiated with ultraviolet light.

In a particularly preferred heat exchanger of the present invention, the surface energy changes by less than 5 %, preferably less than 3 %, when the heat exchanger is treated at a temperature of 70°C with air of 100 % relative humidity for 1250 hours.

The invention encompasses also a preferred embodiment wherein heat exchanger which is combined with a household appliance to form a functional component of the household appliance. More preferred, the household appliance is a dryer, in particular a clothes dryer, comprising the heat exchanger. More preferred as well, the heat exchanger is a heat sink in a process air circuit within the household appliance. In that appliance, the coated surface of the heat exchanger would be exposed to the process air.

The term dryer as used herein not only refers to a dryer as such, but encompasses also a so-called "washer dryer", wherein both washing and drying of laundry is possible.

The invention is of particular use if the dryer comprises a heat pump since the components of a heat pump generally cannot be detached for cleaning the air path. Thus, the tendency to accumulating dirt in the air part of a heat pump should be minimized and the method of cleaning as much as possible simplified for a dryer comprising a heat pump.

The invention is moreover directed to a process for coating a heat exchanger at least partially with a polymer coating on a part of a surface of the heat exchanger, comprising the steps:
(a) pretreating at least the part of the surface to be coated with a polymer coating with a detergent, phosphate and/or borate containing solution,
(b) rinsing the surface with water,
(c) treating the surface with a passivating agent to yield a passivating layer,
(d) rinsing the passivating layer with water, and
(e) coating the passivating layer with a polymer.

In a preferred embodiment of the process according to the invention, the detergent, phosphate and/or borate containing solution in step (a) is either acidic or basic. The use of an acidic or basic (alkaline) liquid is of particular advantage when the heat exchanger comprises or consists of aluminum in that it serves to remove aluminum oxide from the heat exchanger's (fin's) surface.

The solution used in step (a) thus comprises an anionic and/or nonionic tenside, a phosphate and/or borate. As basic agent, for example sodium or potassium hydroxide may be used, in particular sodium hydroxide. Step (a) can be performed by spraying the surface of the heat exchanger with this solution or by immersing the heat exchanger into this solution. The duration of step (a) is preferably up to 3 minutes, more preferably 1 to 2 minutes. The temperature may vary broadly. A preferred temperature range for the treatment in step (a) is from 50 °C to 70 °C.

The rinsing in step (b) is conducted with water, in particular pure water. The pure water can be tap or industrial water that has been purified by distillation or by passing over an ion-exchange resin. Step (b) can be performed by spraying the surface of the heat exchanger with water or by immersing the heat exchanger into water. The duration of step (b) is preferably up to 2 minutes, more preferably up to 1 minute. The temperature may vary broadly. In a preferred embodiment, step (b) can be divided in a step (b1) involving the rinsing with normal water and a step (b2) involving the rinsing with purified water.

The term "rinsing" as used herein is thus used broadly and involves both spraying and immersion.

The water used in step (b) can suitably contain a base or acid. For example, if the solution in step (a) comprises an alkaline substance, it might be advantageous to employ in step (b), in particular in a step (b2) a mixture of water and an acid, for example purified water whose pH is adjusted from 3 to 4 by the addition of sulphuric acid. The sulphuric acid will lend itself to a slight pickling of the surface which will provide for thorough cleaning of the surface and may improve the bond between to surface and the passivating layer that is to be provided subsequently.

In this process, rinsing with water in step (d) is preferably conducted until the water has a conductivity of less than 30 µS/cm.

It is moreover preferred that a drying step (f) is performed between step (d) and step (e). The drying step (f) is preferably performed at a temperature T not exceeding 75 °C, more preferably at a temperature T not exceeding 65 °C. In this manner, particularly good coatings are obtained wherein cracks in the passivating layer are avoided.

In step (c) various passivating agents may be employed. It has been proven of particular advantage, in particular in combination with a heat exchanger comprising at least 90 % aluminum or consisting of aluminum, to use a chromium (III) containing passivating agent. As a result, a thin passivating layer is obtained in general.

The treatment of the surface with a passivating agent in step (c) can be performed by spraying the surface of the heat exchanger with a solution containing a passivating agent or by immersing the heat exchanger into a solution containing the passivating agent. The duration of step (c) is preferably up to 2 minutes, more preferably up to 1 minute. The temperature may vary broadly. A preferred temperature range is however from 25 to 50°C, more preferably from 30 to 40°C.

The rinsing in step (d) of the passivating layer is conducted with water, in particular pure water. The pure water can be water that has been purified by distillation or by passing over an ion-exchange resin. Step (d) can be performed by spraying the surface of the heat exchanger with water or by immersing the heat exchanger in water. The duration of step (d) is preferably up to 2 minutes, more preferably up to 1 minute. The temperature may vary broadly, although it is preferred to use a temperature of less than 50°C, preferably not exceeding 40°C. In a preferred embodiment, step (d) can be divided in several rinsing steps.

In step (e), the passivating layer is coated with a polymer. The coating can be achieved by spraying the passivating layer with a solution containing the coating polymer or by immersing the heat exchanger into a solution containing the coating polymer. Step (e) is generally conducted in less than 1 minute, more preferably less than 30 sec and most preferably not exceeding 10 sec.

In general, the coated heat exchanger obtained in step (e) is allowed to dry. Preferably, the coated heat exchanger is shaken for about 30 seconds to 2 minutes, for example 1 minute, in order to drain off the liquid.

Following the polymer coating, the coated heat exchanger is preferably heated, preferably in a suitable oven, at 250 to 270°C for 20 to 30 minutes, for example for 30 min at 250°C. The coating thus formed strongly adheres to the heat exchanger and depicts a low surface energy not exceeding 40 millinewtons per meter.

It is preferred that step (a) includes removal of grease and oxide compounds from the surface. To this end, it is more preferred that the solution used in step (a) is an alkaline liquid.

An exemplary embodiment of the invention will now be described in detail.

In this embodiment, the dryer has a drying chamber and a closed process air circuit, in which the drying chamber is incorporated and in which a heat pump is provided with a heat sink and a heat source for alternately cooling and heating the circulating process air. The two heat exchangers functioning as heat sink and heat source are embodied in each instance preferably as meandering tube systems, which are soldered together from individual copper tubes and conduit bends and are held in fins arranged one above the other. These fins are thin metal strips made of aluminum and are used to improve the transfer of heat between the working medium flowing through the tube systems and the process air flowing around the tube systems. The heat sink and the heat source are prefabricated in this form and are then inserted into the dryer. The working medium circuit is closed by soldering the heat sink and the heat source using additional conduit pipes.

It is preferred that the surface of a heat exchanger is essentially completely covered by the coating. This is especially true for the case of a dryer, wherein the heat exchanger should be as completely as possible covered everywhere where it can be reached by process air, in particular at any edges present.

The process for coating a heat exchanger at least partially with a polymer coating on a part of a surface of the heat exchanger, comprises a multiplicity of steps:
(a) pretreating at least the part of the surface to be coated with a polymer coating with a detergent, phosphate and/or borate containing solution,
(b) rinsing the surface with water,
(c) treating the surface with a passivating agent to yield a passivating layer,
(d) rinsing the passivating layer with water, and
(e) coating the passivating layer with a polymer.

The detergent, phosphate and/or borate containing solution in step (a) may be acidic or basic. The use of an acidic or basic (alkaline) liquid is of particular advantage when the heat exchanger comprises or consists of aluminum in that it serves to remove aluminum oxide from the surface to be coated. The solution thus comprises an anionic and/or nonionic tenside, a phosphate and/or borate. As basic agent, for example sodium or potassium hydroxide may be used, in particular sodium hydroxide. Step (a) can be performed by spraying the surface of the heat exchanger with this solution or by immersing the heat exchanger into this solution. The duration of step (a) is 1 to 2 minutes. A temperature range for step (a) is set from 50 °C to 70 °C.

The rinsing in step (b) is conducted with pure water. The pure water may be tap or industrial water that has been purified by distillation or by passing over an ion-exchange resin. Step (b) is performed by spraying the surface of the heat exchanger with water or by immersing the heat exchanger into water. The duration of step (b) is up to 1 minute. The temperature may vary broadly. In a preferred embodiment, step (b) can be divided in a step (b1) involving the rinsing with normal water and a step (b2) involving the rinsing with purified water.

The water used in step (b) may suitably contain a base or acid. If the solution in step (a) comprises an alkaline substance, it is advantageous to employ in step (b), in particular in a step (b2), a mixture of water and an acid, namely purified water whose pH is adjusted from 3 to 4 by the addition of sulphuric acid. The sulphuric acid will lend itself to a slight pickling of the surface which will provide for thorough cleaning of the surface and may improve the bond between to surface and the passivating layer that is to be provided subsequently.

Moreover, a drying step (f) is performed between step (d) and step (e). The drying step (f) is performed at a temperature T not exceeding 65 °C. In this manner, particularly good coatings are obtained wherein cracks in the passivating layer are avoided.

In step (c) various passivating agents may be employed. It has been proven of particular advantage, in particular in combination with a heat exchanger comprising at least 90 % aluminum or consisting of aluminum, to use a chromium (III) containing passivating agent. As a result, a thin passivating layer is obtained in general. The treatment of the surface with a passivating agent in step (c) is performed by spraying the surface of the heat exchanger with a solution containing the passivating agent or by immersing the heat exchanger into the solution containing the passivating agent. The duration of step (c) is up to 1 minute. The temperature may vary broadly. A preferred temperature range is however from 30 to 40°C.

The rinsing in step (d) of the passivating layer is conducted with water, in particular pure water. The pure water can be water that has been purified by distillation or by passing over an ion-exchange resin. Step (d) can be performed by spraying the surface of the heat exchanger with water or by immersing the heat exchanger in water. The duration of step (d) is preferably up to 2 minutes, more preferably up to 1 minute. The temperature may vary broadly, although it is preferred to use a temperature not exceeding 40°C. Rinsing with water in step (d) is conducted until the water has a conductivity of less than 30 µS/cm.

The polymer coating is applied by a solution of a polyester-modified methyl phenyl polysiloxane resin combined with a separating substance (which for its part contains nanocrystalline ceramic particles) in an organic solvent, marketed under the name "NP AS 10" by ItN Nanovation AG in Saarbrücken, is used. A pigment is added to the preparation, which fluoresces in visible light when irradiated with ultraviolet light. The preparation is a simple viscous and slightly milky liquid, which is applied by immersing the heat exchanger into it. In this way, the heat exchanger including all edges, in particular all edges of its fins will be covered with the polymer coating. The complete covering of the heat exchanger with the polymer coating can be confirmed by illuminating the coated heat exchanger with ultraviolet light in that the pigment in the preparation fluoresces in visible light. Thus, all areas within the surface of the heat exchanger which should be covered with the coating should fluoresce when the heat exchanger is subjected to ultraviolet light.

As a general remark not limited to the exemplary embodiment, the surface bearing the polymer coating need not necessarily correspond to the complete surface of the heat sink. The coating can be restricted to a part of the total surface on to which the process air blows directly. This part is especially prone to the deposit of foreign particles and in order to save polymer coating material, the coating can be restricted to this area. When used in a dryer, the part of the heat sink to be provided with the polymer coating can in particular be the part, which extends in the flow direction of the process air along the heat sink starting from one of the front sides directly facing the flowing process air over a length between 5 mm and 25 mm. Depending on the application, it may be advantageous to provide corresponding components of the heat sink, for instance fin plates and the like, with the coating prior to their processing and their insertion into the heat sink.

As another general remark not limited to the exemplary embodiment, the coating can optionally extend across the entire heat exchanger or can be restricted to any part, on to which the process air blows during operation. Even if the coating is not applied to the entire heat exchanger it may be of advantage to conduct steps (a) to (d) of the process on the entire heat exchanger in that a passivating layer may render the whole surface resistant to corrosion or any other impairment and allow a stable heat transfer during the lifetime of the heat exchanger. This is particularly true in case of an aluminum heat exchanger where the detrimental effect of any formed aluminum oxide may be avoided.

The present invention provides several advantages. The heat exchanger of the present invention has an excellent resistance to the adhesion of fluff. Even if fluff is deposited on the coated heat exchanger, for example during the operation of a dryer comprising this heat exchanger as a heat sink, it adheres only weakly to the surface of the heat exchanger and can be removed using simple means, in particular by dousing with water. The reliability of an automated cleaning system for the heat exchanger is thus significantly increased and a more stable operation of the heat sink and thus of the dryer, which is not impaired by unwanted deposits, is also ensured over a long period of time.

## Claims

1. Heat exchanger being coated at least partially with a polymer coating on a part of a surface of the heat exchanger, **characterized in that** the part of the surface has a passivating layer interposed between said coating and said surface.

2. Heat exchanger according to claim 1, wherein said passivating layer comprises a chromium compound.

3. Heat exchanger according to claim 2, wherein said chromium compound comprises Cr(III) ions.

4. Heat exchanger according to one of the preceding claims, wherein said coating has a surface energy not exceeding 40 mN/m, in particular not exceeding 30 mN/m.

5. Heat exchanger according to one of the preceding claims, wherein said surface is formed of a metal comprising more than 90 % aluminum, in particular an aluminum alloy.

6. Heat exchanger according to one of the preceding claims, obtainable by a process comprising the steps:
(a) pretreating at least the part of the surface to be coated with a polymer coating with a detergent containing solution,
(b) rinsing the surface with water,
(c) treating the surface with a passivating agent to yield said passivating layer,
(d) rinsing said passivating layer with water, and
(e) coating the passivating layer with said polymer coating.

7. Heat exchanger according to one of the preceding claims, wherein said polymer coating comprises a polysiloxane resin, in particular a polyester-modified methyl phenyl polysiloxane resin.

8. Heat exchanger according to one of the preceding claims, wherein ceramic particles with a size of approximately 50 nm are suspended in said polymer coating.

9. Heat exchanger according to one of the preceding claims, wherein said polymer coating has a thickness of from 1 µm to 50 µm.

10. Heat exchanger according to one of the preceding claims, wherein a pigment that fluoresces in visible light when irradiated with ultraviolet light is suspended in the polymer coating.

11. Heat exchanger according to one of the preceding claims, wherein said surface energy changes by less than 5 % when said heat exchanger is treated at a temperature of 70°C with air of 100 % relative humidity for 1250 hours.

12. Heat exchanger according to one of the preceding claims, which is combined with a household appliance to form a functional component of said household appliance.

13. Heat exchanger according to claim 12, wherein said household appliance is a dryer.

14. Heat exchanger according to one of claims 15 and 16, which is a heat sink in a process air circuit within said household appliance.

15. Heat exchanger according to claim 14, which is incorporated in a heat pump within said household appliance.

16. Process for coating a heat exchanger at least partially with a polymer coating on a part of a surface of the heat exchanger, comprising the steps:
(a) pretreating at least the part of the surface to be coated with a polymer coating with a detergent, phosphate and/or borate containing solution,
(b) rinsing the surface with water,
(c) treating the surface with a passivating agent to yield a passivating layer,
(d) rinsing the passivating layer with water, and
(e) coating the passivating layer with a polymer.

17. Process according to claim 16, wherein in step (d) rinsing with water is conducted until the water has a conductivity of less than 30 µS/cm.

18. Process according to one of claims 16 and 17, wherein a drying step (f) is performed between step (d) and step (e).

19. Process according to claim 18, wherein the drying step (f) is performed at an elevated temperature above a normal ambient temperature, the elevated temperature not exceeding 65 °C.

20. Process according to one of claims 16 to 19, wherein in step (c) the passivating agent contains a chromium compound selected to form Cr(III) ions in the passivating layer.

21. Process according to one of claims 16 to 20, wherein step (a) includes removal of grease and oxide compounds from the surface.

22. Process according to claim 21, wherein the solution used in step (a) is an alkaline liquid.

23. Process according to one of claims 16 to 22, wherein step (b) includes rinsing the surface with water containing sulphuric acid.
